

May 24, 1955

H. CASSMAN ET AL

2,708,788

RENDERING METAL MESHES TAUT

Filed June 1, 1948



Inventors:

Harry Cassman  
William Edward Jeynes  
Reginald Sidney Webley  
By *Joseph O. Ollier*  
Attorney

**1**

2,708,788

**RENDERING METAL MESHES TAUT**

Harry Cassman, Harlington, William Edward Jeynes, Chalvey, Slough, and Reginald Sidney Webley, Hayes, England, assignors to Electric & Musical Industries Limited, Hayes, England, a British company

Application June 1, 1948, Serial No. 30,234

Claims priority, application Great Britain June 3, 1947

4 Claims. (Cl. 29—428)

This invention relates to treating thin metal meshes or foils so as to taunt them, the invention being especially but not exclusively applicable to the treatment of meshes such as employed in the manufacture of television transmission tubes.

In the manufacture of television transmission tubes it is frequently necessary to employ a taut mesh of very fine pitch, as for example when it is desired to evaporate material through the mesh on to a surface so as to form a multiplicity of discrete elements on the surface. Various methods have been proposed for rendering the mesh taut and according to one method a copper mesh is mounted on a frame having a co-efficient of thermal expansion slightly less than the material of the mesh, and it is then heated in vacuo to a temperature of about 600° to 900° C., at which temperature the mesh contracts slowly in relation to the frame and becomes taut, heating being stopped when a suitable degree of tension is attained, which can be judged by experience. It is believed that the contraction of the mesh is due to recrystallisation of the mesh material promoted by the heat treatment. A similar method has been proposed employing a silver mesh mounted on a frame composed of stainless steel or glass. In both cases, however, the method is fairly critical both with respect to the temperature to which the heating is carried, and the time for which it is continued and the success of the method relies to a great extent on the experience of the operator. It seems also that the heat treatment must be carried out in vacuo, though the reason for this is not clear.

The object of the present invention is to provide an improved method of treating thin metal meshes or foils so as to taunt them, with a view to providing a method which is less critical and less dependent upon the experience of the operator.

According to the present invention there is provided a method of treating a thin metal mesh or foil, comprising the steps of extending the mesh or foil on a substantially rigid support, securing the edges of the mesh to the support with the portion of the mesh or foil between the edges thereof free from attachment to the support, applying in contact with said metal mesh or foil a deposit of a metal predetermined to alloy with the metal of the mesh or foil to produce shrinkage thereof, and heating the mesh or foil to cause such alloying to occur with consequent shrinkage of the mesh or foil relative to the support.

The heating may be effected either in air or in vacuo and the alloying of the metals is accompanied by the desired contraction or shrinkage of the mesh or foil, the said contraction or shrinkage occurring at a lower temperature and more rapidly than would otherwise be the case, the alloying of the two metals being believed to be responsible for a more rapid crystal growth in the material of the mesh or foil as it re-crystallises due to the heat treatment. The method is therefore less critical with respect to temperature and time, and in addition, since the alloying of the metals is often accompanied

**2**

by a change in colour, the method may be less dependent upon the experience of the operator. It is also found that in the case of a mesh, for example, subsequent heating as occurs in the usual processes for the manufacture of television transmission tubes is less harmful than in the case of meshes rendered taut by some methods such as employed hitherto, since such subsequent heating does not produce appreciable slackening of the mesh.

In order that the said invention may be clearly understood and readily carried into effect, the same will now be more fully described with reference to the accompanying drawing, in which one example of the present invention, applied to the treatment of a metal mesh for use in the manufacture of a television transmission tube, is diagrammatically illustrated.

Referring to the drawing, a silver mesh 1 having for example 400 filaments per linear inch and a thickness of 0.0004 inch (the mesh being therefore flexible) is cemented to a frame 2 of, for example, stainless steel, by applying a suspension of colloidal silver in oil to the edges of the mesh, applying the mesh to the frame while the mesh is in an extended, that is a more or less taut condition, and subsequently drying out the suspension by heat treatment so that the edges of the mesh are left firmly adhering to the frame 2 by means of a thin layer of silver 3 with the portion of the mesh between its edges free from attachment to the frame as indicated in the drawing. The mesh may of course be secured to the frame in other suitable ways, for example by applying a nickel tape to the edges of the mesh and welding the tape to the frame through the interstices of the mesh. In the drawing the mesh and frame are shown in transverse section, and it will be appreciated that their relative dimensions are not shown in correct proportion. Before or after mounting the mesh on the frame, the mesh is coated with a thin film of gold 4, of a thickness, say, of  $10^{-5}$  inches in the case of a mesh with the dimensions given, the film being applied by any suitable method, for example by plating the gold on to the mesh or by sputtering or evaporating the gold on to the mesh. The mesh secured to the frame is then heated either in air or in vacuo to a temperature of between 300° and 500° C., the heating being continued until the alloying of the two metals is observed, accompanied by a taunting of the mesh. When alloying occurs the colour of the mesh changes from gold to a pale yellow. The invention has been described with reference to the treatment of thin metal meshes so as to taunt them, but the invention can also be applied to the treatment of metal grids or grills such as are employed in other forms of electron discharge devices, or to other arrays of metal filaments which require to be supported in a taut condition. It is to be understood therefore that the expression "metal mesh" used herein and in the claims is intended to include such arrays of metal filaments. In addition the invention may also be applied where it is desired to provide a metal foil supported in a taut condition. Furthermore the method is not limited to the employment of a silver mesh or foil having gold deposited on it, but it can be applied to other metal which will alloy together and produce shrinkage, for example it may be applied to a nickel mesh or foil having copper deposited thereon.

We claim:

1. A method of treating a flexible metal mesh or foil structure suitable for use in an electron discharge device to render it taut, comprising the steps of extending the structure on a substantially rigid support, securing the edges of the structure to the support with the portion of the structure between its edges free from attachment to the support, applying to the surface of said structure a deposit of a metal predetermined to alloy with the metal of the structure to produce shrinkage of the struc-

ture, and finally heating the structure to cause alloying of the metal of said structure with the deposited metal and consequent shrinkage of the unattached portion of said structure relative to said support.

2. A method of treating a flexible silver mesh or foil structure suitable for use in an electron discharge device to render it taut, comprising the steps of extending the structure on a substantially rigid support, securing the edges of the structure to the support with the portion of the structure between its edges free from attachment to the support, applying a deposit of gold to the surface of said structure, and finally heating the structure to cause alloying of the silver of the structure with said gold and consequent shrinkage of the unattached portion of the structure relative to said support.

3. A method of treating a flexible silver mesh suitable for use in an electron discharge device to render it taut, comprising the steps of extending the mesh on a substantially rigid support, securing the edges of the mesh to the support with the portion of the mesh between its edges free from attachment to the support, applying a deposit of gold to the surface of said mesh, and finally heating the mesh to a temperature between 300° C. and 500° C. to cause alloying of the silver of the mesh with said gold and consequent shrinkage of the unattached portion of the mesh relative to the support.

4. A method of treating a flexible silver mesh suitable

for use in an electron discharge device to render it taut, comprising the steps of extending the mesh on a steel frame conforming to a closed figure, securing the edges of the mesh to the frame with the portion of the mesh between its edges free from attachment to the frame, applying a deposit of gold to the surface of said mesh, and finally heating the mesh to cause alloying of said silver and said gold and consequent shrinkage of the unattached portion of the mesh relative to said frame.

References Cited in the file of this patent

UNITED STATES PATENTS

|           |           |                |
|-----------|-----------|----------------|
| 1,106,516 | Lachman   | Aug. 11, 1914  |
| 1,275,022 | Harrison  | Aug. 6, 1918   |
| 1,747,847 | Schlenker | Feb. 18, 1930  |
| 1,863,073 | Smythe    | June 14, 1932  |
| 1,904,241 | Kammerer  | Apr. 18, 1933  |
| 2,162,808 | Gallup    | June 20, 1939  |
| 2,330,202 | Brennan   | Sept. 28, 1943 |

FOREIGN PATENTS

|         |        |               |
|---------|--------|---------------|
| 475,393 | Canada | July 17, 1951 |
|---------|--------|---------------|

OTHER REFERENCES

Barrett, Structure of Metals, page 201, McGraw-Hill Book Company, New York, 1943. (Copy in Div. 3.)